

# UNITED STATES PATENT OFFICE.

ROBERT ABBOTT HADFIELD, OF WESTMINSTER, ENGLAND.

## CAP FOR ARMOR-PIERCING PROJECTILES.

1,375,452.

Specification of Letters Patent. Patented Apr. 19, 1921.

No Drawing.

Application filed May 22, 1920. Serial No. 383,605.

To all whom it may concern:

Be it known that I, Sir ROBERT ABBOTT HADFIELD, baronet, F. R. S., a subject of the King of Great Britain and Ireland, residing at Westminster, England, have invented Improvements in or Relating to Caps for Armor-Piercing Projectiles, of which the following is a specification.

This invention has reference to that kind 10 of caps of conical, conoidal or like shape, for use with armor piercing projectiles, that are made of metal or alloy, such for example as nickel chromium steel, that is capable of being stiffened or hardened and possesses 15 considerable toughness or strength, and the forward end portions of which that will be in front of the point of the projectiles to which such caps are fitted, are made of varying degrees of stiffness or hardness, as 20 described in the specification of Letters Patent No. 1,310,076 with the object of enabling the capped projectile to pass through an armor plate, under varying conditions of impact, without being broken up, or 25 broken up to such an extent as would impair its subsequent proper action.

The present invention has for object to facilitate the manufacture of such caps in a regular and reliable manner so that they 30 shall better fulfil, in a satisfactory manner, the functions which such caps are required to fulfil in practice.

For this purpose a cap made of steel of the kind referred to, after being forged or 35 otherwise formed approximately to the required finished shape, is subjected to the special heat treatment hereinafter described comprising successive heatings and coolings whereby the condition of the steel of which 40 it is made is improved and a special graduated stiffness or hardness is imparted to the cap.

This special heat treatment consists in heating the cap to a high temperature in a 45 furnace, then rapidly cooling it by complete immersion in a cooling medium, such as water or oil, and then gradually withdrawing it, either continuously or in steps or stages, in such a manner that when completely withdrawn it will be at a temperature well below the temperature corresponding to the recalcence point of the steel used but still sufficiently high to evaporate water placed in its interior, the

cap being finally cooled slowly to the ordinary temperature of the atmosphere. It is then reheated in a furnace to a high temperature but below that to which it was previously heated, then allowed to cool to some extent, again reheated but to a lower temperature than on first reheating, and finally again suddenly cooled while still at the maximum temperature, by complete immersion in a cooling medium, such as mentioned. The cap is then finished to shape. The forward end or nose portion of the cap is then heated to a high temperature and the whole cap then dipped, point downward, into a cooling medium, such as water or oil, so as completely to immerse it therein and where it is allowed to remain until practically cold.

A cap made according to the invention may advantageously consist of nickel chromium steel containing under 4% of carbon, 75 about 4% of nickel and about 2% chromium.

Satisfactory results can be attained with a cap made of nickel chromium steel having the following composition, namely about .35% carbon, about 3.88% nickel and about 80 1.80% chromium, when treated in the following manner, after it has been forged or pressed approximately to the required finished shape, namely by slowly heating it in a furnace until it attains a temperature of 85 about 830° C., then cooling it by completely immersing it, point downward, in water or oil and then gradually withdrawing it, either continuously, or in steps or stages, in such a manner that when withdrawn it will 90 be at a temperature well below the temperature corresponding to the recalcence point of the steel used but still sufficiently high to evaporate water placed in its interior, that is to say, a temperature above 100° C., the cap being finally cooled slowly to the ordinary temperature of the atmosphere. It is then reheated in a furnace until it attains a temperature of about 765° to 785° C., then 100 allowed to cool to about 400° C., and again heated up to 600° C., and then again cooled by complete immersion in water or oil.

After this treatment the cap is finished to shape. The forward end portion of the cap is afterward stiffened or hardened by heating the nose portion thereof to a temperature of about 885° to 900° C., as by dipping such nose portion into molten lead, after

which the whole cap is completely immersed in water or oil, point downward, and allowed to remain therein until cold or practically so.

What I claim is:—

- 5 1. The herein described process of producing a steel cap having a stiffened or hardened front end portion for use with an armor piercing projectile, said treatment consisting in heating the cap to a high temperature, then cooling it, first rapidly and afterward more slowly to about the temperature of the atmosphere, reheating it to a high temperature but below that to which it was first heated, allowing it to partly cool, again reheating it but to a lower temperature than the first reheating, then suddenly cooling it, afterward heating its forward end or nose to a high temperature and then cooling the whole cap by completely immersing it point downward in a cooling liquid.
- 10 2. The herein described treatment of a cap made of steel of the character herein referred to, for use with an armor piercing projectile, said treatment consisting in heating the cap to a high temperature, then cooling it by complete immersion in a cooling medium and gradually withdrawing it therefrom, the withdrawal being completely effected while it is at a temperature well below the recalcene point of the steel of which it is composed but still sufficiently high to evaporate water placed in its interior, then allowing it to cool slowly to about the ordinary temperature of the atmosphere, reheating it to a high temperature but below that to which it was previously heated, allowing it to partly cool, again reheating it to a lower temperature than the first reheating, suddenly cooling it while at about the maximum temperature to which it was last reheated, by complete immersion in a cooling medium, afterward heating its forward end or nose to a high temperature and then immersing it completely, point downward, in a cooling

liquid and allowing it to remain there until it is practically cold.

3. The herein described treatment of a cap made of nickel chromium steel, said treatment consisting in heating the cap, after it has been formed approximately to shape, to a temperature of about 830° C., then cooling it by completely immersing it, point downward, in a cooling liquid, then gradually withdrawing it in such a manner that when completely withdrawn it will be at a temperature well below the recalcene point of the steel of which it is composed but above 100° C., finally cooling it slowly to about the ordinary temperature of the atmosphere, reheating it to a temperature of about 765° to 785° C., allowing it to cool to about 400° C., reheating it to a temperature of about 600° C., again cooling it by complete immersion in a cooling liquid, finishing it to shape, and stiffening or hardening its front end portion by heating the nose portion thereof to a temperature of about 885° to 900° C. and completely immersing the cap point downward, in a cooling liquid and allowing it to remain there until it is practically cold.

4. The herein described process of producing a steel cap having a stiffened or hardened front end portion for use with an armor piercing projectile, said treatment consisting in heating the cap to a high temperature, then cooling it, first rapidly to a temperature well below the recalcene point of the steel and afterward more slowly to about the temperature of the atmosphere, subjecting the cap to subsequent tempering treatment and finally heating the forward end or nose to a high temperature and then cooling the cap by completely immersing it in a cooling liquid.

Signed at London in the county of London England this twenty ninth day of April 1920.

ROBERT ABBOTT HADFIELD.